

## UNITED STATES PATENT OFFICE

2,185,809

## ALLOY

Stephen P. Hackley, Stratford, Conn., assignor to The Bridgeport Rolling Mills Company, Bridgeport, Conn., a corporation of Connecticut

No Drawing. Application February 17, 1939,  
Serial No. 256,863

## 1 Claim. (Cl. 75—157)

The present invention relates to an alloy, particularly of the bronze type, and has for an object the production of an alloy having the characteristics of toughness, workability, spring quality and high electrical conductivity, and in which such uniformity may be maintained that it may be relied upon to perform satisfactorily under all conditions, and in its various applications.

It is also proposed to provide an alloy which has ductility, and which may be subjected to repeated cold rolling to produce predetermined tempers without intermediate anneals. It is also an object to provide an alloy which will be relatively unaffected by prolonged heat at temperatures to which it may be subjected when in normal use.

The alloy according to the invention is especially applicable to the production of products demanding these characteristics, for instance electrical switches, fuse clips, plug receptacles, and the like, springs, sash chain, baggage hardware, etc. Tinned alloys heretofore employed for the particular uses contemplated herein have been found to be subject to such variation and uncertainty when they are worked, that the products fabricated from such alloys cannot always be depended upon to perform their intended functions.

The alloy according to the invention consists of a mixture of copper, zinc, tin, and a small quantity of manganese, added as a flux. In preparing the alloy the ingredients are mixed in about the following proportions: copper 87 to 90 percent; zinc 9 to 13 percent; tin 2 to 4 percent. These ingredients are melted in a crucible and a small amount of manganese is added as a flux. The proper amount of manganese may be determined empirically, but in any case is relatively small, for example less than 2 percent.

The alloy may be cast in bars and thereupon rolled into strips or sheets, or may be extruded and drawn into rods or other desired shapes. It

is suitable for any purpose where toughness is desired, and is especially desirable where spring qualities are demanded, or where the metal is subjected to deformation in use. It has been found to have much higher electrical conductivity than other tinned alloys usually recommended for similar purposes, and is therefore especially useful in the manufacture of electrical devices.

The alloy has ductility. In practice it has been found that at 5#s hard—that is, when rolled five Brown & Sharpe numbers successively, and without intermediate anneals—the alloy averages about 83,000 lbs. per square inch in tensile strength with an elongation of 9 percent in 2 inches, while at 11#s hard, it has an average tensile strength of around 100,000 lbs. per square inch with an average elongation of 6.6 percent in 2 inches. These figures are from tests employing a stock of .066 rolled to the two tempers cited.

The alloy is practically unaffected when subjected to prolonged heat, tests having indicated that after heating for hours at 250° C. it showed greater hardness under a Rockwell B scale test.

As compared to other alloys intended for similar uses which have been found to be temperamental and undependable, the alloy according to the invention has been found to have absolute uniformity in all tempers and in its various applications, so that it can be relied upon to perform characteristically under all conditions.

Having thus described my invention what I claim is:

A cold workable alloy characterized by its toughness, ductility, spring quality, high tensile strength, and high electrical conductivity, composed of copper in the amount of 87 to 90 percent, zinc in the amount of 9 to 12 percent, tin in the amount of 2 to 4 percent, and manganese added as a flux in an effective amount not in excess of 2 percent, and said alloy being substantially free of other constituents.

STEPHEN P. HACKLEY.